

E. C. WASHBURN,  
CASTING APPARATUS,  
APPLICATION FILED MAR. 21, 1912.

1,192,024.

Patented July 25, 1916.



Fig. 1.

Fig. 2.



WITNESSES

*W. C. Washburn*  
*Ed. C. Washburn*

INVENTOR

*E. C. Washburn*

BY

*DuBoisfield & Drue*  
ATTORNEYS

# UNITED STATES PATENT OFFICE.

EDWIN C. WASHBURN, OF ENGLEWOOD, NEW JERSEY.

## CASTING APPARATUS.

1,192,024.

Specification of Letters Patent. Patented July 25, 1916.

Application filed March 21, 1912. Serial No. 685,157.

To all whom it may concern:

Be it known that I, EDWIN C. WASHBURN, a citizen of the United States, residing at Englewood, in the county of Bergen and State of New Jersey, have invented certain new and useful Improvements in Casting Apparatus, of which the following is a full, clear, and exact description, such as will enable others skilled in the art to which it appertains to make and use the same.

This invention relates to molding, and with respect to its more specific features, to a molding apparatus suitable for use in casting of various kinds.

One of the objects of the invention is to provide a practical device of the kind described which shall insure a highly homogeneous product.

Another object of the invention is to provide a simple and efficient device which shall prevent piping in a product.

Another object of the invention is to provide a simple and efficient device of the kind described which shall substantially prevent piping and control segregation in the resultant product.

Another object of the invention is to provide a heat insulating device which may be readily applied to various kinds of molds.

Another object of the invention is to provide a practical and efficient process for the casting of various materials whereby a highly desirable product is obtained.

Other objects will be in part obvious and in part pointed out hereinafter.

The invention accordingly consists in the several steps and the relation and order of one or more of such steps with relation to each of the others thereof, and in the features of construction, combinations of elements and arrangement of parts, which will be exemplified in the method hereinafter disclosed and the construction hereinafter set forth, and the scope of the application of each of which will be indicated in the following claims.

In the drawing, wherein is shown one of the various possible embodiments of the invention, Figure 1 represents a cross-section on the line  $\alpha$ — $\alpha$  of Fig. 2; and Fig. 2 represents a longitudinal sectional elevation showing an ingot in place.

Similar reference numerals refer to similar parts throughout both views of the drawing.

As conducive to a clearer understanding

of this invention it is pointed out that in casting, segregation of elements and unequal contraction of parts may occur whereby imperfections such as pipes are produced in the body of the finished product. For example, in casting steel ingots, during the cooling stage there are apt to be segregations of slag, silicon, phosphorus and sulfur in various parts of the ingot, and more particularly in that part which retains the greatest amount of heat to the end of the cooling period. Piping also occurs in these steel ingots generally following the line of slowest cooling, and usually takes the form of conical-shaped cavities extending from the top face of the ingot approximately along its longitudinal axis toward the center. In rolling these ingots and in further treatment for the production of various articles, this portion of the ingot through which the pipe extends and in which a large portion of the segregation occurs should be cut off and perhaps recast, or else if the portion be retained in the ingot and an article made therefrom, structural weakness will be found in the article. This condition in castings is hence a highly undesirable one, and this invention seeks, among other things, to do away with this piping and segregation and the various other evils attendant thereupon.

It has been found, in accordance with the present invention, that if the chamber of a molding device be provided with a heat insulating portion whereby one portion of the chamber may be preserved at a relatively higher temperature than other portions of the chamber, the segregation of materials, phenomena in the nature of piping, and other undesirable features, may be substantially overcome.

Referring now more particularly to the drawing, 1 represents a tubular upright ingot mold or molding chamber. The chamber is provided with refractory walls 2, the inner periphery of which tapers from the upper part of the chamber toward the lower part. Disposed about the chamber 1 and held within by the inner walls thereof is a preferably removable heat-insulating device comprising a plurality of insulating members; one an outer, preferably annular, member 3, composed of sand or other suitable material, and the other an inner, preferably annular, hollow metallic member 4, preferably made of iron. The member 4 is

concentric with the ring 3. The member 4 is adapted to provide a continuous closed air space which serves as an insulating medium, acting in this capacity in conjunction with the sand ring 3 which also constitutes an insulating medium. The annular member 3 is preferably provided on its inner periphery with a facing of carbonaceous material, preferably graphite, 5.

10 It will be noted that the sand ring 3 is preferably shaped to contact with the inner walls of the chamber 1 and is held thereby. This heat insulating device may be conveniently formed by molding the sand ring 15 about the inner metallic ring and baking the two, whereby the sand adheres to the iron ring and forms a hard outer coating. The facing of carbonaceous material may then be put upon the inner periphery of the 20 sand.

In the use of the device the heat insulating member is inserted within the chamber 1, being positioned therein so that the upper or neck portion of the metal will be 25 surrounded by and contact with the ring 3. The metal, designated as 6, is then poured into the mold until the upper portion thereof is a little below the upper surface of the ring 3. The pouring is then discontinued. 30 With steel and like casting, the upper surface of the molten material is then preferably covered or sprinkled with carbonaceous material 7. The steel or other material used should be preferably in a quiet state 35 when cast, and to accomplish this in the case of steel, silicon or similar material may be added thereto. The use of a quiet steel insures the retention of the carbonaceous material in proper position with respect to the metal. The 40 carbonaceous materials 5 and 7 burn when brought in contact with the metal, and thus provide hot insulating coverings for the metal. The metal is then allowed to cool. During 45 the course of the cooling, the impurities, including slag, silicon, phosphorus and sulfur will tend to segregate in that portion of the chamber which is hottest and there will also be a tendency for the metal to cool more quickly in the outer parts thereof than in 50 the inner. As a consequence, the portions of the metal below the heat insulating device will tend to cool more rapidly than the neck portion of the material which is contained within the space inclosed by the annular 55 members 3 and 4, due to the fact that the sand acts as an insulation, as does also the air within the hollow chamber in the member 4 and prevents the heat from radiating from that part of the metal. By thus keeping 60 this portion heated to a higher temperature than the outer portions, the impurities will tend to segregate there. The contraction of metal in the cooler portions will cause a flow of metal from the neck portion 65 downward through the center of the mold,

and the molten material in the neck portion will gradually and uniformly sink downward until the whole inner portion of the ingot has undergone a contraction in accordance with the final temperature reached. 70 Thus the resultant product instead of showing pipes and segregations will have only a small cupped neck portion in which most of the impurities will have segregated and which may be broken off with very little loss 75 of metal.

In actual practice ingots have been obtained in which the proportion of metal forming the cup and including the impurities was about two per cent. of the ingot. In 80 these ingots there was substantially no piping.

It will be seen, in accordance with the construction outlined, that by providing a removable refractory heat insulating ring a 85 convenient device is provided for use in connection with a number of chambers, for as soon as one of the ingots, for example, in a given chamber, has cooled partially, the ring may be withdrawn therefrom and made 90 ready for further casting. It is to be noted in this connection that by providing the chamber 1 with tapering inner walls, means is thereby provided for securely supporting the refractory insulating member. It is to 95 be understood that the insulating ring may occupy any convenient position in the mold, that is, it may be placed in such position that a casting, occupying only half the chamber or any other proportion thereof, is 100 formed.

It is to be further noted that the annular ring serves as a guide for the metal which is being poured into the molding chamber and directs the stream so that it is substantially prevented from contacting with the walls of the chamber, thus precluding the formation of flakes of metal on the sides of the chamber by sudden cooling, through contact of the stream of metal therewith. This 105 flake formation on the sides of the wall, if the metal be not directed away therefrom, will accumulate upon the outer surface of the finished ingot. This accumulation, however, is prevented, as noted, by guiding the 110 stream by means of the insulating member.

It will also be noted in accordance with the construction outlined that the heat contained in the metal below the annular refractory member will tend to pass off 115 through this member and will thereby impart a certain proportion of heat thereto. By thus heating the annular refractory member the rate of transference of heat to the metal held within the space inclosed thereby will be materially lessened and thus the efficiency of the insulating device will be increased.

It is pointed out that the mold 1 is placed with its larger diameter at the top, thereby 120

providing a slower cooling in the upper portion and acting thus in conjunction with the insulating device to keep the upper portion of the metal hot.

5 Although it has been convenient to describe this process in connection with the molding of ingots, it is to be understood that it is equally applicable to the various processes of casting.

10 It is also intended to be understood that the term "casting" used herein is intended in its broad sense as indicating the treatment of molten material by means of suitable devices, to give it a desired shape.

15 The device described is a very efficient one, is simple and practical and may be used on almost any kind of mold. It is easily handled and may be replaced without difficulty and at small expense. It will thus be seen that the device fulfills, among others, 20 the objects enumerated in a highly practical manner.

As many changes could be made in carrying out the above method, and in the above 25 construction, and many apparently widely different embodiments of this invention could be made without departing from the scope thereof, it is intended that all matter contained in the above description or shown 30 in the accompanying drawings shall be interpreted as illustrative and not in a limiting sense.

It is also to be understood that the language used in the following claims is intended to cover all of the generic and specific 35 features of the invention herein described, and all statements of the scope of the invention which, as a matter of language, might be said to fall therebetween.

40 Having described my invention, what I claim as new and desire to secure by Letters Patent is:

1. A molding device comprising an upright tubular chamber and an annular refractory member adapted to surround heated material held in said chamber, said annular member incasing a hollow metallic ring having air therein.

2. A molding device comprising an upright tubular chamber provided with tapered walls, an annular refractory member adapted to be supported by said walls on the inner periphery of said chamber, said annular refractory member comprising an inner hollow metallic ring having air there-

in, and an outer sand ring inclosing said metallic ring.

3. In an apparatus of the kind described, in combination, a chamber adapted to receive metal therein, an annular refractory member provided with a carbonaceous coating on the inner periphery thereof adapted to be set within said chamber, and carbonaceous material adapted to be sprinkled on the surface of the metal held within said chamber.

4. A heat insulating device comprising a plurality of annular members, one of said members including refractory material and another of said members provided with an inclosed hollow chamber.

5. A heat-insulating device comprising an annular refractory member incasing a metallic ring providing an air space there- 75 within.

6. A heat-insulating device comprising an annular refractory member comprising an inner hollow metallic ring providing a continuous air-space and an outer sand ring inclosing said metallic ring.

7. A device of the nature disclosed comprising a molding chamber and a removable heat insulating device resting thereon, said heat insulating device comprising an inner portion serving as a form and providing an air space therewithin, and refractory material molded about said form.

8. A device of the nature disclosed comprising a molding chamber and a heat insulating device, said heat insulating device comprising an inner annular metallic member provided with a closed air space therewithin, and sand molded about said annular member.

9. A device of the nature disclosed comprising a molding chamber and a removable heat insulating member resting on the interior periphery below the upper edge thereof, said heat insulating member comprising an inner annular hollow metallic ring, and sand molded about said ring in a shape to conform to the inner periphery of said molding chamber.

In testimony whereof I affix my signature, in the presence of two witnesses.

EDWIN C. WASHBURN.

Witnesses:

J. B. L. ORME,  
HELEN M. SEAMANS.